

## [54] JET FUEL MANUFACTURE

[75] Inventors: **Kenneth L. Dille**, Wappingers Falls; **George S. Saines**, Fishkill; **Alfred Arkell**, Wappingers Falls, all of N.Y.

[73] Assignee: **Texaco Development Corporation**, New York, N.Y.

[22] Filed: **Oct. 13, 1970**

[21] Appl. No.: **80,481**

[52] U.S. Cl. .... **208/49, 208/15, 260/666 P, 260/666 PY, 260/667**

[51] Int. Cl. .... **C07c 5/10**

[58] Field of Search ..... **208/15, 49; 260/666 P, 666 PY, 667**

## [56] References Cited

## UNITED STATES PATENTS

|           |         |                    |           |
|-----------|---------|--------------------|-----------|
| 3,161,016 | 12/1964 | Smith et al. ....  | 260/666 P |
| 3,533,938 | 10/1970 | Leas.....          | 208/15    |
| 3,105,351 | 10/1963 | Stahly.....        | 260/666 P |
| 3,113,425 | 12/1963 | Smith et al. ....  | 260/666 P |
| 3,128,597 | 4/1964  | Smith et al. ....  | 260/666 P |
| 3,183,278 | 5/1965  | Koch.....          | 260/677   |
| 3,274,276 | 9/1966  | Louvar.....        | 260/671   |
| 3,317,611 | 5/1967  | Louvar et al. .... | 260/671   |
| 3,412,165 | 11/1968 | Slaugh et al. .... | 260/667   |

## OTHER PUBLICATIONS

Appleby et al. "Symposium On Jet Fuels," Preprint of

the American Chemical Society, Division of Petroleum Chemistry, New York, N.Y., Vol. 5, No. 4, Sept. 1960 pages C-31 to C-38.

Primary Examiner—Herbert Levine

Attorney—Thomas H. Whaley, Carl G. Reis and Robert A. Kulason

## [57] ABSTRACT

Jet fuels which have both a high heat content and an acceptable low temperature viscosity are prepared by the hydroalkylation of mononuclear aromatic hydrocarbon fractions. Benzene, toluene, and Udex extract, and mixtures thereof, are the preferred starting materials. These are hydroalkylated by reaction at about 30°-250° C. under super-atmospheric pressures of about 20-70 atmospheres of hydrogen, thus producing hydroalkylates containing cycloalkyl-substituted benzenes, methylcyclohexyl-substituted toluenes and the like. These are further reduced to the corresponding cycloalkyl-substituted cyclohexanes, together with methylcyclohexyl methylcyclohexanes and methylcyclohexane when toluene is used, and the reduction products are adjusted to a final desired heat content and low temperature viscosity by stripping off or adding methylcyclohexane. The preferred catalyst is finely divided nickel on a support containing both a zeolite and a silica-alumina cracking catalyst.

3 Claims, No Drawings

## JET FUEL MANUFACTURE

This invention relates to a method for the production of jet fuels of high heat content from mononuclear aromatic hydrocarbons such as benzene, alkylbenzenes such as toluene, ethylbenzene and the like, and dialkylbenzenes such as the various xylenes, including mixtures thereof such as those obtained in Udex extracts.

A principal object of the invention is to convert these aromatic hydrocarbons into jet fuels by hydroalkylation processes. A further object is the production of jet fuels, having both a high heat content and an acceptable low temperature viscosity, by reducing cycloalkyl-substituted mononuclear aromatic hydrocarbons to a mixture of cycloalkyl-substituted cyclohexanes.

A still further object of the invention is the provision of new jet fuels wherein the principal heat-producing ingredients are cyclohexyl-substituted benzenes, methylcyclohexyl-substituted toluenes and other mononuclear aromatic hydrocarbon derivatives and their reduction products such as dicyclohexyl-substituted cyclohexanes, polycyclohexyl cyclohexanes and mixtures thereof together with sufficient methylcyclohexane to impart a desired low temperature viscosity.

Additional objects of the invention will become apparent from the following description of the principles thereof when taken with the attached examples and the appended claims.

It is well known that the turbojet engine operates by the combustion of fuel between an air compressor and a turbine, thereby increasing the volume and temperature of the air so that the work of compression can be taken out of the gases by the turbine with enough energy remaining to impart the high final kinetic energy and speed to the jet that is needed for propulsion. For this purpose a fuel having a high heat content, as measured by its heat of total combustion, is needed. In addition, a fuel having an acceptable low temperature viscosity is needed because of the low temperatures which may be encountered during storage and high altitude use.

We have found that jet fuels having both of these properties can be obtained by processes based on the hydroalkylation of mononuclear aromatic hydrocarbons such as benzene, toluene, higher alkylbenzenes, xylenes and the like, including particularly mixtures of these hydrocarbons such as are obtained by extracting aromatic petroleum fractions with suitable solvents. In the preferred practice of our invention these hydrocarbons or hydrocarbon mixtures are hydroalkylated, thereby producing mixtures containing cycloalkyl-substituted mononuclear aromatic hydrocarbons, followed by partial or complete reduction to the corresponding cycloalkyl-substituted cyclohexanes or alkylcyclohexanes. We have found that jet fuels having varying but controlled ratios of heat content to low-temperature viscosity can be obtained by fractionating the reduction products so obtained, or by stripping volatile ingredients such as methylcyclohexane therefrom.

The production of cycloalkyl aromatic compounds by hydroalkylation is a known procedure. It is carried out by reacting mononuclear aromatic hydrocarbons such as benzene, toluene and mixtures thereof with hydrogen in the presence of a mixed catalyst which contains both an alkylation component and a hydrogenation component. Typical catalysts and reaction condic-

tions are described in U. S. Pat. Nos. 3,274,276 and 3,317,611, and any of the catalysts and reaction conditions described in these patents may be used in practicing our present invention. We have found, however, that good results are obtainable by carrying out the hydroalkylation in the presence of a finely divided nickel catalyst supported on a substantially alkali metal-free mixture of a zeolite, from which substantially all of the alkali metal has been removed, together with a silica-alumina cracking catalyst of the type now employed for the vapor phase cracking of petroleum hydrocarbons into gasoline. This catalyst has the advantage that it can also function as a hydrogenation catalyst in the second stage of our process wherein the hydroalkylate is reduced by further reaction with hydrogen. Alternatively, a more efficient hydrogenation catalyst, such as Ni on alumina, may be used during second stage reduction.

In the preferred practice of our invention the hydroalkylation is preferably carried out at temperatures below about 450° F. and preferably within the range of about 110° to 400° F. and pressures of hydrogen of about 20-70 atmospheres. The subsequent reduction of the hydroalkylate may be obtained by continuing the reaction with the same or other hydrogenation catalyst at about 300 to 1,000 p.s.i. and temperatures below 450° F. until the uptake of hydrogen is substantially complete. As a practical matter pressures of hydrogen of about 450 to 550 p.s.i. are preferred in order to lessen the reaction time. The resulting reaction mixture is then preferably distilled at atmospheric or sub-atmospheric pressures to strip off unreacted or partially reacted starting materials and by-products of relatively low heat content.

We have found, as a result of the tests shown in the following specific examples, that the heat of combustion on both a weight and a volume basis is increased by increasing the number of cyclohexyl substituents on phenyl and also on tolyl and other alkylphenyl groups. In contrast to this, the heat of combustion on a volume basis is increased with an increase in the number of cyclohexyl groups attached to cyclohexane and alkyl cyclohexanes, but on a weight basis the heat of combustion is decreased. In both cases, however, the poly-substituted compounds have relatively high heat of combustion values. These discoveries are important in the production of jet fuels for specific end uses, such as for military planes on the one hand and commercial planes on the other hand. In military jet fuels the heat content is preferably based on the volume of the fuel, because most military applications are volume limited. In commercial jet airplanes the fuel value is evaluated on a weight basis, since space is not so important, and therefore a high heat of combustion on a weight basis is preferred. It is an important advantage that the process of our invention can be adapted to produce jet fuels of either type from relatively inexpensive starting materials such as benzene, toluene, and alkylbenzene mixtures obtained by the solvent extraction of aromatic hydrocarbon fractions. A particularly useful source of such mixtures is Udex extract, obtained by the selective extraction of aromatics from various feed stocks by absorption in aqueous diethylene glycol solutions, and the use of such extracts as starting materials constitutes a particular specific feature of the invention.

In its most practical aspect, therefore, the preferred practice of our invention consists in treating toluene or toluene-containing mixtures such as Udex extract to a

3-stage process. In the first stage the toluene is hydroalkylated as described above to a product containing methylcycloalkyl-substituted toluenes, which are usually mixed with unconverted toluenes since the hydroalkylation is seldom carried to completion. In the second stage this product mixture is reduced by hydrogenation to form the corresponding methylcycloalkyl-substituted methylcyclohexanes along with methylcyclohexane from the toluene reduction. In the third stage a part or all of the methylcyclohexane is removed by distillation in order to adjust the jet fuel product to the desired final viscosity and B.T.U. content. Alternatively, most of the unconverted toluene from the first stage can be stripped off for recycle to the hydroalkylation unit. Using this procedure there is no excess methylcyclohexane produced during second stage reduction. Jet fuel blends with energy contents in the 136,000 B.T.U. per gallon range are obtained by either of these procedures, and viscosities as low as 50-75 poises at minus 65° C. are obtainable by the presence of about 20 percent to about 50 percent of methylcyclohexane in the product. Such blends may contain dicyclohexylbenzene, tricyclohexylbenzene, dicyclohexyl cyclohexane or higher polycyclohexyl cyclohexanes, but usually mixtures of two or more of these compounds are present in ratios that will vary with the extent of hydroalkylation and of reduction used in the process.

The invention will be further described and illustrated by the following examples. The catalyst used in these examples consisted of about 6 percent by weight of finely divided nickel distended on about 94 percent of a hydrocarbon-cracking catalyst support which was a substantially alkali metal-free mixture of about 22 percent by weight of a modified zeolite Y, about 58 percent of silica and about 20 percent of alumina.

The modified zeolite portion of the cracking component has uniform pore openings of from 6-15 Angstrom units, has a silica-alumina ratio of at least 2.5, e.g. 3-10, and has a reduced alkali metal content. The modified zeolite is prepared by subjecting synthetic zeolite Y to ion exchange by contacting the zeolite several times with fresh solutions of an ammonium compound at temperatures ranging between about 100° and 250° F. until it appears that the ion exchange is substantially complete. The ion exchanged zeolite is then washed to remove solubilized alkali metal and dried at a temperature sufficiently high to drive off ammonia. This converts the zeolite Y to the hydrogen form and reduces the alkali metal content to about 2-4 weight per cent. The ion exchanged zeolite is then calcined at a temperature of about 1,000° F. for several hours. After cooling, the ion-exchanged calcined zeolite is subjected to additional ion exchange by contact several times with fresh solutions of an ammonium compound and again washed and dried. This treatment results in a further reduction in the alkali metal content of the zeolite to less than 1 percent and usually to about 0.5 percent. It would appear that after the first calcination, it is possible to engage in further ion exchange with the removal of additional alkali-metal ions not removable in the initial ion exchange. Calcination at e.g. 100°-1,200° F. may take place here or it may be postponed until after the incorporation of the amorphous inorganic oxide and impregnation with the hydrogenating component at which time the composite should be calcined. Whether calcination is postponed or re-

peated, the final calcination temperature should not exceed 1,200° F.

The silica-alumina portion of the support is a composite of alkali metal-free silica and alumina of the well-known type used in petroleum cracking and described, for example, in U. S. Pat. No. 2,469,314. It is frequently prepared by acidifying an aqueous sodium silicate solution with aqueous 25% sulfuric acid, washing the resulting hydrated silica free from alkali metal salts, suspending it in aluminum sulfate solution, precipitating with ammonia, filtering and washing. The filter cake is preferably mixed with a sufficient quantity of the modified zeolite to obtain 22 percent by weight of zeolite after drying and the mixture is dried and calcined. It is then impregnated with 6 percent of nickel by adding nickel nitrate solution, drying and heating in the presence of hydrogen.

#### EXAMPLE 1

a. Toluene was mixed with about 5 percent of its weight of the above-described catalyst and hydroalkylated at 375° F. and about 500 p.s.i.g. hydrogen pressure. After 1.5 hours a 31 percent conversion was obtained with 79 percent of the hydroalkylate being mixed isomeric methylcyclohexyltoluenes.

b. In a second run, 4.5 grams of the catalyst were suspended in 47 grams of toluene in a 100 c.c. rocking autoclave and hydroalkylation was continued under the same reaction conditions for 5 hours at which point the toluene conversion was over 90 percent.

The reaction mixture was fractionated by distillation at 1 torr; i.e., at 1 millimeter of mercury pressure. A total of 17.3 grams of methylcyclohexane and unconverted toluene was first removed. A second cut, taken at 48°-50° C., consisted of 11.9 grams of mixed methylcyclohexyltoluenes. A third cut weighing 2.1 grams distilled over at 120°-127° C. and contained polysubstituted compounds as the principal ingredients.

c. Following these preliminary investigations a larger scale run was made with 460 grams of toluene in a 1-liter rocking autoclave at 370°-380° F. and 500 p.s.i.g. pressure using 22.5 grams of the same catalyst. This run was carried out to high conversion and the product was distilled under the conditions and with the results shown in the following table.

TABLE I

| Distillation | Cut       | Wt. |       |                                                                |
|--------------|-----------|-----|-------|----------------------------------------------------------------|
| Press.       | Temp. °C. | No. | Grams | Products <sup>1</sup>                                          |
| Atm.         | 110       | 1   | 199   | Toluene & traces of MChA                                       |
| 20 Torr      | 145       | 2   | 103   | Mixed MCHT's                                                   |
| 8 Torr       | 121-123   | 3   | 42    | Mixed MCHT's                                                   |
| 1 Torr       | 106-108   | 4,5 | 7     | and higher                                                     |
|              |           |     | 22    | substitution products                                          |
|              |           |     |       | 1. MChA = Methylcyclohexane; MCHT's = Methylcyclohexyltoluenes |

#### EXAMPLE 2

Run (c) of Example 1 was repeated, using the same temperature and pressure conditions and the same quantities of toluene and catalyst, but the product mixture was further reduced with hydrogen to give the corresponding reduction products. These were separated by distillation into a first cut weighing 279 grams and consisting of methylcyclohexane with traces of toluene, a second cut weighing 118 grams and composed of 84 weight per cent of dimethylcyclohexanes and 16 weight per cent of methylcyclohexyltoluenes, and a res-

idue weighing 14 grams and containing higher substitution products.

### EXAMPLE 3

Using the same catalyst, reaction conditions and rocking autoclave as in Example 2, 390 grams of benzene was hydroalkylated and reduced to give the following main distillation fractions.

TABLE II

| Cut  | Temp. (°C.) | Pressure (torr) | Products                   |
|------|-------------|-----------------|----------------------------|
| 1    | 78          | Atm.            | cyclohexane                |
| 2    | 83          | 4.0             | dicyclohexane              |
| 4    | 123         | 0.5             | dicyclohexylcyclohexane    |
| res. |             |                 | polycyclohexylcyclohexanes |

These materials, as well as some of those from the toluene series were reserved for subsequent tests.

Runs were also made at 370°-380° F. and 500 p.s.i.g. with o-xylene, m-xylene and p-xylene, using the same catalyst in an amount of 11% on the weight of the hydrocarbon. Hydroalkylation and reduction were obtained with all three of the starting materials but the hydrogen uptake rate was greater with the meta and para xylene than with orthoxylene.

### EXAMPLE 4

Udex extracts are principally mixtures of mononuclear aromatic hydrocarbons obtained by selective extraction of aromatic-containing feed stocks with aqueous diethylene glycol solution. A typical extract may contain 15.3 volume per cent of benzene, 40.4 per cent of xylenes and ethyl benzene and 42.5 per cent of toluene. They are a very attractive source of raw material for conversion into jet fuels because of their abundance and relatively low cost.

A sample of Udex extract was used which was free

10

6

TABLE III

| Cut     | Temp. (°C.) | Pressure (torr) | Products                                              |
|---------|-------------|-----------------|-------------------------------------------------------|
| 1,2     | 96-175      | Atm             | Starting mixture and corresponding reduction products |
| 3       | 125         | 8               | mono-substitution products                            |
| residue |             |                 |                                                       |

### EXAMPLE 5

#### Production of Jet Fuels

We have found that jet fuels which have both a high 15 heat content and an acceptable low temperature viscosity can be prepared by the hydroalkylation and reduction procedures illustrated in Example 1-4. By varying the composition of the mononuclear aromatic hydrocarbons and their mixtures from benzene to alkylated benzenes, and by controlling the degree of cycloalkylation and subsequent, hydrogenation of the remaining aromatic ring, it is possible to control the aromatic to naphthenic ratio.

This control allows the synthesis of fuels having properties which adapt them for specific end uses. Thus, for example, jet fuels which have higher aromatic ratios are better suited for military use due to their higher density while lower density fuels for commercial aircraft are obtained by hydrogenation of the aromatic ring which may be followed by light end stripping if desired.

The hydroalkylation products of benzene, toluene and Udex extract and their reduction products were evaluated as jet fuel ingredients, in comparison with methylcyclohexane and i-propylidicyclohexyl, by determining their heats of combustion and their viscosities at minus 65° F. The results with benzene hydroalkylation products are shown in the following table.

TABLE IV

| Test number | Compound, mixture or blend                                          | B.t.u./lb. | Density, g./cc. | B.t.u./gal. | -65° F. viscosity, poise |
|-------------|---------------------------------------------------------------------|------------|-----------------|-------------|--------------------------|
| 1           | i-Propylidicyclohexyl                                               | 18,420     |                 | 136,544     |                          |
|             | Methylecyclohexane                                                  | 18,569     | .7688           | 119,140     |                          |
| 2           | Cyclohexylbenzene (CHB)                                             | 17,504     | .9473           | 138,054     |                          |
| 3           | Di-CHB's <sup>1</sup>                                               | 17,736     | .9719           | 143,537     |                          |
| 4           | Di-CHB's <sup>1</sup> plus 20 weight percent MCHA <sup>2</sup>      | 17,905     | .9217           | 137,740     | >163                     |
| 5           | Di-CHB's <sup>1</sup> plus 25 weight percent MCHA <sup>2</sup>      | 17,929     | .9189           | 137,500     | <58                      |
| 6           | Tri-CHB's <sup>1</sup>                                              | 17,844     | .9848           | 146,340     |                          |
| 7           | Dicyclohexane                                                       | 18,478     | .8838           | 136,000     |                          |
| 8           | Dicyclohexylcyclohexane                                             | 18,312     | .9277           | 141,600     |                          |
| 9           | Dicyclohexylcyclohexane plus 22 weight percent MCHA <sup>2</sup>    | 18,299     | .8918           | 136,200     | ≈163                     |
| 10          | Polycyclohexylcyclohexanes                                          | 18,218     | .9629           | 146,090     |                          |
| 11          | Polycyclohexylcyclohexanes plus 40 weight percent MCHA <sup>2</sup> | 18,238     | .8788           | 133,770     | ≈163                     |
|             | Polycyclohexylcyclohexanes plus 50 weight percent MCHA <sup>2</sup> | 18,328     | .8570           | 131,100     | <58                      |

<sup>1</sup> Methylcyclohexane (MCHA).

<sup>2</sup> Cyclohexylbenzenes (CHB's).

from butanes and contained 90-95 percent aromatics, mostly toluene and higher alkylated benzenes. Gas chromatographic analysis showed that it contained at least six different compounds and, after hydroalkylation, the product mixture contained at least ten components in the monosubstitution region.

The sample was mixed with 5.3 percent of its weight of catalyst and hydroalkylated at 370°-380° F. using 500 p.s.i.g. of hydrogen pressure. The rate of hydrogen uptake was slightly less than that of pure toluene but was greater than for the xylenes of Example 3. Distillation gave the following results.

The dicyclohexylbenzenes reported in this table were made by hydroalkylation of benzene mixed with 5 percent of its weight of the catalyst previously described. Distillation of the hydroalkylate gave dicyclohexylbenzenes as a fraction boiling within the range of 150°-165° C. at 1 torr pressure. The tricyclohexylbenzenes used were obtained from the same materials in a rocking autoclave run, the desired fraction (cut 5; boiling range 158°-185° C. at 0.5 torr) containing only a trace of dicyclohexylbenzenes. The dicyclohexylcyclohexane and polycyclohexylcyclohexanes were the products of Table II of Example 3. Runs 7-11 show that

jet fuels having both high heat contents and acceptable viscosities at low temperatures can be obtained by blending a mixture of polycyclohexylcyclohexanes with about 20 percent to about 50 percent of their weight of methylcyclohexane.

Table IV shows that increasing the number of cyclohexyl groups on benzene (compare 1,2 and 5) increases the heat of combustion on both a weight and volume basis. In contrast to this, increasing the number of cyclohexyl groups on cyclohexane (compare 6, 7 and 9) causes the heat of combustion on a weight basis to decrease and on a volume basis to increase. In both cases, the trisubstituted compounds have relatively high heat of combustion values of over 146,000 BTU's/gal., but the dicyclohexylbenzenes are better suited for military purposes because of their higher density. Test Nos. 3 and 4 show that their low temperature viscosities can be brought into the desired range by blending them with minor proportions of methylcyclohexane.

Table V shows the results with products of Examples 1, 2 and 4 with isopropyldicyclohexyl as a basis of comparison.

has distinct viscosity and cost advantages over the latter compound.

The foregoing tables show that the hydroalkylation products of mononuclear aromatic hydrocarbons have heats of combustion in the 135,000 to 146,000 BTU/gal. range, but their flow properties at minus 65° F. require improvement if they are to be used for military purposes. According to Air Force specifications, the desired viscosity for a jet fuel is 5 poise at -65° F. However, it is evident that higher viscosities would be acceptable if the fuel had an unusually high heat value or very low cost. Sheldyne, for example, has a viscosity of 170 poise at -65° F., high heat value of 150,000 BTU/gal., and an unrealistically high cost of \$42.00/gal. Using the 170 poise value as a guide, two polymer standards were obtained which had viscosities of 163 and 58 poise at room temperature. The Blends shown in Table IV were made in order to meet or improve on the Sheldyne viscosity without too great a loss in heat content. Methyl cyclohexane (MCH) was used as the diluent both because the Air Force has expressed an interest in MCH from the standpoint of cost, availability, and heat-sink capacity and because it is a reduction

TABLE V

| Test number | Compound or mixture           | Source                    | B.t.u./lb. | Density, g./cc. | B.t.u./gal. | -65° F. viscosity, poise |
|-------------|-------------------------------|---------------------------|------------|-----------------|-------------|--------------------------|
| 1           | i-Propyldicyclohexyl          | Ex. 1(c), cut 2           | 18,430     | 0.9311          | 136,844     | Solid                    |
| 2           | Methylcyclohexyltoluenes      | Ex. 1(c), cut 4,6         | 17,658     | 0.9311          | 136,880     |                          |
| 3           | Higher subst. products        | Ex. 1(c), residue         | 17,643     | 0.9314          | 136,850     |                          |
| 4           | Higher subst. products        | Ex. 1(c), residue         | 17,606     | 0.9721          | 142,520     |                          |
| 5           | Me-cyclohexyl-me-cyclohexane  | Ex. 2, cut 2              | 18,363     | 0.8837          | 135,150     | ≈163                     |
| 6           | Di-subst.-me-cyclohexane      | Ex. 2, residue            | 18,063     | 0.9291          | 139,670     |                          |
| 6           | Mixture from Udex extract run | Ex. 4, cut 3 plus residue | 17,708     | 0.9321          | 137,450     |                          |

Although the heat contents of the blends shown in Table IV have been decreased, compared to the parent materials, they are still in the range of 131,000 BTU/gal. to 137,500 BTU/gal. A comparison of the most promising blends with materials being considered by the Air Force is shown in the following summary:

| Components                           | BTU/gal. | Viscosity (Poise at -65° F.) | Cost (\$/gal.) |
|--------------------------------------|----------|------------------------------|----------------|
| Air Force (Targets)                  | 160,000  | 5                            | 0.25           |
| Sheldyne                             | 150,000  | 170                          | 42.00          |
|                                      |          |                              |                |
| i-propyldicyclohexyl                 |          |                              |                |
| Me-cyclohexane (MCHa) (From benzene) | 119,000  |                              | 0.25           |
| DCHB's                               | 143,500  | All less than                | 1.00           |
| + 25 wt.% MCHa                       | 137,500  | <58                          | "              |
| Tricyclohexanes                      | 141,500  |                              |                |
| + 22 wt.% MCHa (From Toluene)        | 136,200  | ≈ 163                        | "              |
| dimethyl-dicyclohexane               | 135,100  | ≈ 163                        | "              |

136,500 (F.P. -29° F.)

Note that the tricyclohexanes have a higher heat content (141,500 BTU/gal.) than the structurally similar and commercially available isopropyldicyclohexyl (136,500 BTU/gal.). Tricyclohexanes blended with 22 wt. percent methylcyclohexane have a heat content almost the same as isopropyldicyclohexyl and the blend

product of toluene that can be obtained in practicing the process of our present invention.

#### EXAMPLE 6

We have found that toluene can be converted into mixtures that, from the standpoint of energy content, viscosity, cost and ease of manufacture, are outstanding as jet fuels. This is done by a three-stage process wherein (1) toluene is hydroalkylated to a product containing methylcycloalkyl-substituted toluenes, usually in admixture with unconverted toluene, (2) this product mixture is reduced by hydrogenation to form the corresponding methylcycloalkyl-substituted methylcyclohexanes along with methylcyclohexane from toluene reduction, and (3) a part or all of the methylcyclohexane is removed by distillation in order to adjust the jet fuel product to the desired final viscosity and BTU content. Alternatively, most of the unconverted toluene from the first stage can be stripped off for recycle to the hydroalkylation unit. This procedure eliminates the production of excess methylcyclohexane during second stage reduction.

Jet fuel blends with energy contents in the 136,000 BTU per gallon range, including the higher energy polysubstituted products, 139,700 BTU/gal., from the hydroalkylation-reduction stages, with viscosities less than 170 poises at -65° F. and with a substantial cost advantage over existing jet fuels are obtained by this procedure. The process also has the flexibility of providing jet fuel blends with a range of energy-viscosity properties that can be controlled simply by varying the

amount of methylcyclohexane removed from the mixture of reduction products.

It will thus be seen that the objects set forth above, among those made apparent from the preceding description, are efficiently attained and, since certain changes may be made in carrying out the above method and in the composition set forth without departing from the scope of the invention, it is intended that all matter contained in the above description shall be interpreted as illustrative and not in a limiting sense.

What we claim is:

1. A method of producing a jet fuel having both a high heat content and an acceptable low temperature viscosity which comprises

a. hydroalkylating a charge hydrocarbon mononuclear aromatic hydrocarbon composition containing as reactant at least one component selected from the group consisting of benzene, toluene, xylenes, and ethylbenzene by reacting said reactant at 110° F-450° F and pressure of 20-70 atmospheres in the presence of hydrogen and hydroalkylating catalyst to produce a hydrocarbon hydroalkylate containing a cycloalkyl-substituted mononuclear aromatic hydrocarbon;

b. reducing said cycloalkyl-substituted mononuclear aromatic hydrocarbon in said hydroalkylate at temperature below 450° F and at pressure of 300-1000 psi thereby forming a reduced hydroalkylate containing as by-product reduced charge mononuclear aromatic hydrocarbon which has been reduced to mononuclear cyclohexanes; and

5 c. separating at least a portion of the by-product mononuclear cyclohexanes from said reduced hydroalkylate thereby forming as product a jet fuel characterized by a high heat content and an acceptable low temperature viscosity.

2. A method of producing a jet fuel having both a high heat content and an acceptable low temperature viscosity which comprises

10 hydroalkylating a charge hydrocarbon composition containing toluene by reacting said toluene at 110° F-450° F and pressure of 20-70 atmospheres in the presence of hydrogen and hydroalkylating catalyst at hydroalkylation conditions to produce a hydrocarbon hydroalkylate containing methylcyclohexyl toluenes and unreacted toluene; reducing said hydroalkylate at temperature below 450° F and at pressure of 300-1000 psi thereby forming a reduced hydroalkylate containing methylcyclohexyl-methyl cyclohexanes and by-product methyl cyclohexanes; and separating at least a portion of said by-product methyl cyclohexanes from said reduced hydroalkylate thereby forming as product a jet fuel characterized by a high heat content and an acceptable low temperature viscosity.

25 3. A method of producing a jet fuel as claimed in claim 2 wherein said separation is effected to yield a product jet fuel containing about 20-50 percent of methylcyclohexane.

30 \* \* \* \* \*

35

40

45

50

55

60

65

UNITED STATES PATENT OFFICE  
CERTIFICATE OF CORRECTION

Patent No. 3,773,652 Dated November 20, 1973

Inventor(s) KENNETH L. DILLE, GEORGE S. SAINES and ALFRED ARKELL

It is certified that error appears in the above-identified patent  
and that said Letters Patent are hereby corrected as shown below:

[73] "Texaco Development Corporation" should read  
--Texaco, Inc.--

Col. 1, line 67 "condic-" should read --condi- --

Col. 7, lines 46-48 The chemical formula should be in  
the lefthand column under "Shelldyne".

Col. 7, line 54 The phrase "All less than" should be in  
the right hand column above the entry  
"1.00".

Signed and sealed this 11th day of June 1974.

(SEAL)

Attest:

EDWARD M. FLETCHER, JR.  
Attesting Officer

C. MARSHALL DANN  
Commissioner of Patents